

1,374,434.

C. G. COLLINS.  
PROCESS OF TREATING ORE.  
APPLICATION FILED JAN. 13, 1920.

Patented Apr. 12, 1921.



**INVENTOR**

CALEB G. COLLINS  
BY  
Wallace White  
ATTORNEY

# UNITED STATES PATENT OFFICE.

CALEB G. COLLINS, OF WOODMERE, NEW YORK, ASSIGNOR TO C. AMORY STEVENS, OF NEW YORK, N. Y.

## PROCESS OF TREATING ORE.

1,374,434.

Specification of Letters Patent.

Patented Apr. 12, 1921.

Application filed January 13, 1920. Serial No. 351,221.

To all whom it may concern:

Be it known that I, CALEB G. COLLINS, a citizen of the United States of America, residing at Woodmere, county of Nassau, 5 State of New York, have invented a new and useful Process of Treating Ore, of which the following is a specification.

My invention relates to the separation of metal from the ore and consists in a novel 10 method of treating the ore, by the use of which a greater yield of metal is obtained from the ore when the ore is afterward subjected to the usual air or wet methods of concentration.

15 The object of my invention is to treat the ore in such a way as to remove the air and the moisture therefrom, and to insure that the air and moisture will not reenter the ore once freed, as a preliminary treatment to 20 the ore before it is subjected to the concentration process. The utilization of this method of preparing the ore has the result that a heavier ore, freed of its air and moisture, is provided at the commencement of 25 the concentration process, resulting in a better separation, due to the greater density of the ore, when subjected to the usual concentration process.

My process consists first in heating the 30 ore to such a temperature as will cause all the air and moisture to be driven out from the ore, and this temperature is preferably between 300° and 500° Fahrenheit. While the ore is being thus heated, I prefer to agitate it so as to secure a uniform heating, and afford every chance for the air and moisture to be driven out from every particle of the ore. When the ore has been 35 thoroughly dried, and all the air driven out, and preferably while it is still in heated condition, I treat the ore with material to prevent the reentry of the air and moisture. This material may be any substance of very 40 fine nature which will penetrate into the pores of the ore, such as crude oil, or even finely powdered material such as powdered charcoal. I prefer to use a crude oil that will pass into a vapor upon coming into contact with the heated ore, as I find that this 45 gives excellent results. After this material has been spread upon the ore, and during the spreading action, I prefer to agitate the ore continuously so as to afford an opportunity for the material to reach every particle of the ore.

When the ore has been treated in this manner, it may be concentrated by any of the usual methods; and the concentration of the ore does not fall in the scope of this invention. Ores that are subjected to this 60 preliminary treatment before concentration, however, are found on concentration to give a materially increased yield of metal; and particularly is this true in the case of ores containing chlorids and bromids. 65

In order that my process may be fully understood, I have illustrated in the accompanying drawing a form of apparatus in which it may be carried out, it being understood that this is only one form of apparatus 70 suitable for the purpose, and that the process may be performed in other suitable devices.

Referring to this drawing, I provide a furnace 1 preferably having a slightly inclined chamber 2 covered by an arch 3, at one end of which is the combustion chamber 4 wherein fuel may be burned upon the grate 5 to produce the heat required, the combustion gases passing through the chamber 2 and escaping by a chimney 7. 75

Mounted in a position slightly inclined preferably to correspond with the incline of the chamber 2, is a vessel 8 preferably in the form of a tube mounted at each end externally of the furnace upon suitable means such as wheels 9 so that it may be rotated. 80

Opening into the higher end of the tube 8 there may be provided means such as the funnel 10 for inserting the ore to be treated, and this ore, due to the incline of the tube 8, and its rotation upon the wheels 9, is agitated within the tube, and under the influence of gravity gradually passes from the higher to the lower end thereof, and is discharged from the lower end into a receiving chamber 11 from which the treated ore may be removed by suitable means such as the screw 12. 90

In the form of apparatus shown it is proposed to use crude oil for closing up the pores of the ore to prevent the reentry of air and moisture after the heating has been accomplished, and the means for spraying the ore with the oil may comprise a pipe 13 extending inside the tube 8, and provided with a plurality of openings 14 adapted to sprinkle the oil upon the ore. 100

The operation of the device may be continuous, the oil being fed in by the funnel 110

10 and gradually passing through the tube 8 as the tube is rotated, the rotation causing agitation of the ore so as to afford an opportunity for all the moisture and air to be  
5 driven from it, while the ore is being heated; and the rate of rotation of the tube 8 may be so regulated to control the passage of the ore through the tube that the ore will be adequately heated and the moisture  
10 and air fully driven off by the time the ore reaches the portion of the pipe 13 containing the holes 14 for supplying the oil to the ore. Further agitation of the ore as it passes through the remaining portion of  
15 the tube 8 causes the oil to be well distributed, and to thoroughly close up the pores of the ore so as to prevent any air or moisture getting into them. As the ore reaches the lower end of the tube 8, it is discharged into the container 11, whence it  
20 may be removed for the usual concentration process.

Having now described my invention, I claim and desire to secure by Letters Patent:  
25 1. The method of preparing ore, which consists in heating the ore to drive off air and moisture, and treating it with material to prevent the reentry of air and moisture, and thereafter concentrating the ore.

2. The method of preparing ore which 30 consists in subjecting the ore to heat sufficient to drive off the air and moisture, and spraying the ore with a liquid that will vaporize on reaching the heated ore, the vapors filling the pores of the ore, thereby 35 preventing reentry of air and moisture; and thereafter concentrating the ore.

3. The method of preparing ore which consists in heating the ore to a temperature of from 300° to 500° Fahrenheit, and treating the heated ore with material to prevent 40 reentry of air and moisture, and thereafter concentrating the ore.

4. The method of preparing ore which consists in passing the ore through a heated zone, agitating the ore during passage, and treating the heated ore with material to prevent 45 reentry of air and moisture, and thereafter concentrating the ore.

5. The method of preparing ore which 50 consists in heating the ore to drive off air and moisture, and spraying the heated ore with crude oil, and thereafter concentrating the ore.

In testimony whereof I have signed my 55 name to this specification.

CALEB G. COLLINS.